

**1**

3,809,604

**PROCESS FOR FORMING A FLUFFED  
FIBROUS PULP BATT**

Phillip Waite Estes, Aiken, S.C., assignor to Riegel  
Textile Corporation, New York, N.Y.  
No Drawing. Filed Aug. 2, 1972, Ser. No. 277,280  
Int. Cl. D21d 3/00

U.S. CL. 162—100

2 Claims

**ABSTRACT OF THE DISCLOSURE**

A process for forming a fluffed fibrous pulp batt for use in sanitary products wherein the fluffed fibrous pulp batt has markedly improved strength and integrity with longer, stronger and more uniform fibers for producing greater loft, moisture absorption and strength in the batt. The process includes the continuous steps of treating of the wet pulp to effect kinking and interlocking of the fibers, forming the fibers into a wet pressed pulp sheet, drying, mechanically fiberizing the sheet and air-laying the debonded kinked fibers to form a fluffed pulp batt with improved strength and integrity due to the kinked and interlocked fiber formation. Preferably, the process also includes the steps of producing a dilute, aqueous slurry of the kinked and interlocked fibers and incorporating in the slurry a cationic debonding agent, so that minimum breakage of the fibers will result during the mechanical fiberizing step due to the debonding effect of that cationic debonding agent, and a fluffed pulp batt will be produced with minimum fiber breakage therein.

This invention relates to a process for improving a fluffed fibrous pulp batt adapted for use in sanitary products or the like wherein the fluffed fibrous pulp batt has markedly improved strength and integrity with longer, stronger and more uniform fibers for producing greater loft, moisture absorption and strength in the batt.

In sanitary products, such as sanitary napkins, diapers, etc., fluffed fibrous pulp batts have been utilized as the core material for providing absorbency and other characteristics in the sanitary products. These fluffed fibrous pulp batts are normally produced by manufacturing a wet pressed pulp sheet formed by conventional pulp and paper making processes and then mechanically fiberizing the wet pressed pulp sheet into individual fibers and air-laying the individual fibers to form a fluffed fibrous pulp batt which may be cut and placed into the center or core of the sanitary products.

In such fluffed fibrous pulp batts, the fluffed fibrous pulp batt must have the properties of strength and integrity inasmuch as the batt is utilized as the core or center of the sanitary products and must therefore provide strength and integrity to the overall sanitary products. Also, it is desirable to have minimum fiber breakage from the mechanical fiberizing operation so that the ultimate air-layed fluffed fibrous pulp batt will provide improved moisture absorption characteristics. Also, it is desirable for the wet pressed pulp sheet to be substantially completely fiberized to eliminate undesirable residual un-fiberized sheet particles and minimize fiber dust so as to provide longer, stronger and more uniform fibers for producing greater loft and strength in the batt.

Accordingly, it is the object of this invention to provide a process for improving a fluffed fibrous pulp batt adapted for use in sanitary products or the like wherein the fluffed fibrous pulp batt has markedly improved strength and integrity with longer, stronger and more uniform fibers for producing greater loft, moisture absorption and strength in the batt.

It has been found by this invention that the above object may be accomplished by providing a process com-

**2**

prising the continuous steps of treating wet pulp fibers for effecting kinking and interlocking of the fibers, forming the fibers into a wet pressed pulp sheet, drying, mechanically fiberizing the sheet and air-laying the debonded kinked fibers to form a fluffed pulp batt with improved strength and integrity due to the kinked and interlocked fiber formation. Preferably, the process also includes the steps of producing a dilute, aqueous slurry of the kinked and interlocked fibers and incorporating in the slurry

- 10 a cationic debonding agent, so that minimum breakage of the fibers will result during the mechanical fiberizing step due to the debonding effect of the cationic nature and a fluffed pulp batt will be produced with minimum fiber breakage therein.
- 15 By any conventional pulp making and paper making technique, the fibers produced are essentially non-kinked. That is, they exist as straight fibers in the wood and after going through cooking and bleaching process, are delivered to the paper making machine in essentially an unkinked form. Then, when they are formed into a sheet and dried, they are held in place by the structure of the sheet and essentially remain unkinked fibers in the dry sheet. Then, as in the case of fiberizing pulp, they are broken apart by mechanical means, the individual fibers obtained are still essentially unkinked. The air-laid batt formed of these fibers has relatively little strength and integrity. There is no bonding between dry fibers once separated and brought back into contact with one another and any type of stresses put on the batt, such as handling, 20 or pulling, easily slides the fibers by one another resulting in breakage of the pad structure and the sanitary product utilizing the batt.

Referring now to the specific steps of the process of this invention, the present invention is applicable to practically all conventional types of pulps made in conventional manner by well-known kraft, soda, sulfite or neutral sulfite processes. The raw material, that is the fibers to be pulped, and otherwise processed in accordance with this invention, may be any one or more of the various types of cellulosic materials commercially used in paper and paperboard manufacture. Illustrative examples are wood, cotton, linters, flax, hemp, ramie, bagasse, esparto fiber pulps, etc. Generally speaking, it is desirable to use relatively long fiber material for ultimate individual fiber strength and for high resistance to breaking, powdering or dusting when subjected to fiberizing treatment.

Wet pulp fibers, of the above type, are treated for effecting kinking and interlocking of the fibers. This treating step for effecting kinking and interlocking of the fibers may be effected by the use of a mechanical kinking device, such as described in Hill et al. U.S. Pat. 2,516,384, issued July 25, 1950. The device of this patent is one example of a suitable device for treating wet pulp fibers for effecting kinking and interlocking of the fibers and any device that mechanically kinks wet fibers may be utilized within the context of this invention. In order to effect kink wet fibers, they should be dewatered to some extent and the kinking operation may include a separate dewatering step such as a screw press, or apparatus may be used that both dewatering and works the fibers into kinks with one operation. Such a combination action is produced in a "Curlator" machine and is described in the section entitled "The Curlator," pages 258-261, Pulp and Paper Manufacture, volume 2, 1st Edition, 2nd Impression published by McGraw-Hill Book Company, Inc. in 1951.

Next, a dilute, aqueous slurry of the kinked and interlocked fibers is produced, a cationic debonding agent is incorporated into the slurry and the slurry is formed into a wet pressed pulp sheet and dried.

Suitable cationic debonding agents are disclosed in Hervey and George U.S. Pats. Re. 26,939, issued Aug. 18, 1970; 3,554,862, issued Jan. 12, 1971; and 3,554,863,

issued Jan. 12, 1971, all of which are assigned to the assignee of the present invention. These debonding agents may be generally classified as cationic long chain fatty alkyl compounds having at least twelve carbon atoms in at least one alkyl chain.

Depending upon the type of paper or board making machinery used, the desired speed of operation, and the desired degree of impregnation of the kinked fibers with the chemicals or debonding agent, the debonding agent is incorporated into the wet slurry of kinked fibers at the stock chest or head box of the paper or paperboard machine. A suitable type of Fourdrinier paper machine and the process of forming paper thereon is disclosed in Bedwell U.S. Pat. 2,488,700, issued Nov. 22, 1949; and a suitable type of cylinder paper machine is disclosed in Edge U.S. Pat. 2,005,839, issued June 25, 1935. Reference may be had to these patents for a disclosure of paper machines and processes of operation suitable for use in the present invention.

The amount of debonding agent added to the wet slurry of fibers will vary within specific ranges with the type of pulp used. Reference may be had to the above three patents, assigned to the assignee of the present invention, for these specifics.

After formation of a dried, wet pressed pulp sheet, the sheet is mechanically fiberized into individual debonded kinked fibers and air-laid to form a fluffed pulp batt. The mechanical fiberizing is performed with a minimum of fiber breakage due to the debonding effect of the cationic agent. The resulting fluffed pulp batt has a minimum of fiber breakage and substantially improved strength.

A suitable machine for mechanically fiberizing and air-laying is disclosed in George U.S. Pat. 3,543,351, issued Dec. 1, 1970, and assigned to the assignee of the present invention.

Thus, it may be seen that the combination of treating of wet pulp fibers for effecting kinking and interlocking of the fibers and incorporating into a slurry of such kinked and interlocked fibers a cationic debonding agent produces a unique and novel wet pressed pulp sheet which may be mechanically fiberized and air-laid with minimum breakage of fibers due to the debonding effect of the cationic agent and which forms a fluffed pulp batt with substantially improved strength and integrity due to the kinked and interlocked fiber formation.

It is an object of the present invention to provide a pulp sheet which is formed by the combination of kinking and interlocking of the fibers and incorporating into a slurry of such kinked and interlocked fibers a cationic debonding agent, and which may be mechanically fiberized and air-laid with minimum breakage of fibers due to the debonding effect of the cationic agent and which forms a fluffed pulp batt with substantially improved strength and integrity due to the kinked and interlocked fiber formation.

It is a further object of the present invention to provide a pulp sheet which is formed by the combination of kinking and interlocking of the fibers and incorporating into a slurry of such kinked and interlocked fibers a cationic debonding agent, and which may be mechanically fiberized and air-laid with minimum breakage of fibers due to the debonding effect of the cationic agent and which forms a fluffed pulp batt with substantially improved strength and integrity due to the kinked and interlocked fiber formation.

In the specification there has been set forth a preferred embodiment of the invention and, although specific terms are employed, they are used in a generic and descriptive sense only and not for purposes of limitation.

What is claimed is:

1. A process for forming a fluffed fibrous pulp batt for use in sanitary products, said process comprising the continuous steps of mechanically treating of web pulp fibers for effecting kinking and interlocking of the fibers, producing a dilute, aqueous slurry of the kinked and interlocked fibers, incorporating in the slurry a cationic debonding agent, forming the wet slurry into a wet pressed pulp sheet, drying the sheet, mechanically fiberizing said sheet, and air-laying the debonded kinked fibers to form fluffed pulp batt with minimum fiber breakage and substantially improved strength and integrity due to the kinked and interlocked fiber formation.

2. A process for forming a fluffed fibrous pulp batt for use in sanitary products, said process comprising the continuous steps of mechanically treating of wet pulp fibers for effecting kinking and interlocking of the fibers, forming the kinked fibers into a wet pressed pulp sheet, drying the sheet, mechanically fiberizing the sheet, and air-laying the fiberized kinked fibers to form a fluffed pulp batt with substantially improved strength and integrity due to the kinked and interlocked fiber formation.

#### References Cited

#### UNITED STATES PATENTS

|           |         |                 |           |
|-----------|---------|-----------------|-----------|
| 3,395,708 | 8/1968  | Hervey et al.   | 162—179 X |
| 3,171,773 | 3/1965  | Estes et al.    | 161—168   |
| 2,516,384 | 7/1950  | Hill et al.     | 162—100   |
| 3,556,931 | 1/1971  | Champaigne      | 162—158   |
| 3,370,590 | 2/1968  | Hokanson et al. | 162—158 X |
| 3,617,439 | 11/1971 | Chapman         | 162—158   |
| 3,554,862 | 1/1971  | Hervey et al.   | 162—158   |
| 3,554,863 | 1/1971  | Hervey et al.   | 162—158   |

40 ROBERT L. LINDSAY, JR., Primary Examiner

A. L. CORBIN, Assistant Examiner

U.S. CL. X.R.

45 128—284, 162—158

UNITED STATES PATENT OFFICE  
CERTIFICATE OF CORRECTION

Patent No. 3,809,604 Dated May 7, 1974

Inventor(s) Phillip Waite Estes

It is certified that error appears in the above-identified patent  
and that said Letters Patent are hereby corrected as shown below:

Column 1, line 17, after "includes" delete --includes--

Column 1, line 56, change "ultime" to --ultimate--

Column 2, line 55, change "effecting" to --effectively--

Column 4, line 8, change "web" to --wet--

Column 4, line 10, change "interlocker" to --interlocked--

Signed and sealed this 10th day of September 1974.

(SEAL)

Attest:

MC COY M. GIBSON, JR.  
Attesting Officer

C. MARSHALL DANN  
Commissioner of Patents